

July 28, 1925.

1,547,984

W. WEBER

MEANS OF TREATING AMMONIUM CHLORIDE LIQUORS IN IRON CONTAINERS

Filed Aug. 6, 1923



Inventor:  
Walter Weber  
By James L. Morris  
Attorney

## UNITED STATES PATENT OFFICE.

WALTER WEBER, OF DUSSELDORF, GERMANY.

## MEANS OF TREATING AMMONIUM-CHLORIDE LIQUORS IN IRON CONTAINERS.

Application filed August 6, 1923. Serial No. 656,099.

*To all whom it may concern:*

Be it known that I, WALTER WEBER, a citizen of Germany, residing at 10 Kasernenstrasse, in the city of Dusseldorf, Germany, **5** have invented certain new and useful Improvements in Means of Treating Ammonium-Chloride Liquors in Iron Containers, of which the following is a specification.

This invention has reference to means for **10** the protection of the container walls of iron or of equivalent material in the manufacture and in the treatment of ammonium-chloride solutions or liquors, and my invention relates particularly to improvements **15** upon the procedure outlined in my previous application for U. S. Patent Serial 626155 of March 19, 1923. In this prior application I have described a process for the treatment of liquors containing ammonium-chloride in iron containers in which these liquors are treated by means of an iron anode with **20** a weak continuous current which leaves the apparatus through the iron walls thereof.

It is obviously essential for the efficient **25** protection of the containers against the iron dissolving properties of liquors containing ammonium-chloride that the electric current be uniformly distributed along the entire iron wall of the container which constitutes **30** the anode. In carrying out my invention aside of other iron vessels a plurality of vaporizers provided with tubular heaters or radiators may be utilized. It therefore becomes necessary to subdivide the positive **35** side of the admission of current in the well known manner, in order to be able to adapt it to the iron surfaces to be protected by electrical means, so as to produce a uniform cathodic current density. The mere subdivision **40** of the anodic admission of current, however, does not yet result in an absolutely reliable uniformity of intensity of current in all portions. Particularly with the commercial sorts of iron employed as anode material which contain varying proportions of **45** foreign substances according to their source of production, a lack of uniformity in the distribution of the current upon the several anodes is likely to occur; and the material **50** of the anodes will be consumed to great disadvantage very much more rapidly than with an amount equivalent to the electric current.

In view of these facts my present invention **55** relates to means for the practising of substantially the same process, described in

my previous application, but adapted to produce the required uniformity in the distribution of the current, and in the rate of dissolution of the iron anode. **60**

Such means are shown on the accompanying drawing by way of example in a conventional manner, the drawing illustrating a form of apparatus embodying the principles of my invention. The apparatus comprises **65** essentially a plurality of anodes of iron bars mounted in the evaporating vessels, so as to produce a uniform distribution of the current, the said anodes being surrounded by a protective tubing consisting of electrically **70** insulating material and within which the anodes may be axially reciprocated, the arrangement being such that the anodes will come in contact at their end portions only with the liquors containing ammonium chloride. As an electrically insulating material **75** I may make use, for instance, of hard rubber or porcelain. The anode bars are preferably shifted in the protecting tube at a rate corresponding to the desired rate of **80** flow of the current through the individual anode bar in proportion to its solubility corresponding to the rate of flow of the electric current, that is to say, on an average one gramme per ampere-hour. **85**

Where there is lack of uniformity in the distribution of the current an anode through which there is an excessive rate of flow of current will be consumed at a rate greater than that at which it is axially shifted, in **90** consequence whereof the terminal portion of the anode bar which is in contact with the liquors will recede more and more into the interior of the protective tube. This causes a progressive increase of the resistance **95** which must be overcome by the electric current. On the other hand, an electrode through which the rate of flow of the current is too low will be consumed at a rate less than that at which it is axially shifted. **100** The extremity of the iron bar which is in contact with the liquors in this case will therefore, project more and more from the protective tubing, so that the resistance to the electric current is progressively diminished. **105**

This positively acting displacement in proportion to the resistance constitutes a self-regulation of the strength of current, and produces in operation a uniform rate of **110** flow of current through the individual anodes, by which means that a uniform dis-

tribution of current on the iron surface to be protected is obtained. Furthermore, the consumption of iron of the anode in this method of operation corresponds almost exactly to the minimum quantity theoretically required.

In the accompanying drawing an evaporator of the Robert-type is shown by way of example, and it is to be understood that a plurality of such evaporators with, say 107½ sq. feet (10 square meters) heating surface each may be used. The bodies of these evaporators are connected to the negative terminal of a regulatable direct current dynamo of from 2 to 4 volts pressure, and are provided with five iron anodes A connected in parallel connection with one another and also connected to the positive terminal of the source of current. The anodes consist, for instance, of round iron bars of, say, 0.59 inch (15 millimeters) diameter, and are contained, as shown in the drawing, in tubes B of hard rubber or the like. The tension of the dynamo is regulated in such a manner that a current of 50 amperes is caused to flow for each evaporating unit; that is to say with four units there is a total current strength of 200 amperes. The several anode bars A are moved through the tubes B toward the liquor at the rate of about 0.3 inches (¾ centimeters) an hour. After the operation is continued for a short time only a uniform rate of flow of 10 ampere per anode has been obtained. The several round iron bars are 29½ inches (750 millimeters) long and are screw threaded at both ends so that they may be extended by being screwed together and may, in this manner, be completely used up without remnant.

The invention has been described and shown only by way of example and is not restricted to any particular form of apparatus or manner of execution. It is to be understood that changes and modifications may be made therein to better adapt the invention to varying conditions without deviating from the spirit of my invention as set forth in the claims hereunto appended.

60 I claim:—

1. The method of treating liquors containing ammonium chloride with an electric current, which consists in passing a weak electric current through a plurality of iron

anodes each having one of its ends in contact with said liquor and causing said anodes to move longitudinally into the liquor at a speed corresponding to the rate of solution of the anodes when the flow of the current therethrough is at the desired 60 amperage, whereby the current flow is maintained at a substantially constant value.

2. The method of treating liquors containing ammonium chloride with an electric current, which consists in passing an electric current through a plurality of iron anodes each having one of its ends in contact with said liquor, and causing said anodes to move longitudinally into said liquor at a speed corresponding to the rate 70 of solution of said anodes when the flow of current therethrough is at the rate of ten amperes per anode, whereby such current flow is maintained at a substantially constant value.

3. In an apparatus of the character described, an iron evaporating container, a plurality of iron anodes spaced apart and extending into said container, and insulating protecting tubes surrounding said anodes, said anodes being longitudinally movable into said container at a speed corresponding to the rate of solution of the anodes when the flow of the current therethrough is at the desired amperage, whereby said current flow is maintained at a substantially constant value.

4. In an apparatus of the character described, an iron evaporating container, a plurality of iron anodes mounted in said container and longitudinally movable to maintain their extremities in contact with the liquor contained in said container, and tubes of insulating material surrounding said anodes.

5. In an apparatus of the character described, an iron liquor containing evaporating container, a plurality of axially movable extensible iron anodes mounted in said container, and provided with threaded ends 100 and having their inner ends adapted to contact with the liquor contained in said container, and insulating tubes surrounding said anodes and insulating said tubes from said container.

In testimony whereof I have hereunto set my hand.

WALTER WEBER.